

Nov. 11, 1941.

M. FAIRLIE ET AL

2,262,528

LUBRICATION

Filed July 15, 1938



INVENTORS  
Matthew Fairlie  
Leonard E. Beare  
BY

Dennis, Davis, Macmillan and Leonard  
ATTORNEYS

## UNITED STATES PATENT OFFICE

2,262,528

## LUBRICATION

Matthew Fairlie and Leonard E. Beare, Hammond,  
Ind., assignors to Sinclair Refining Company,  
New York, N. Y., a corporation of Maine

Application July 15, 1938, Serial No. 219,458

11 Claims. (Cl. 123—196)

This invention relates to lubrication and particularly to lubrication employing petroleum-base oils. The invention aims to prolong the useful life of such oils, inhibit formation of "carbon," sludge, tars, asphaltenes, and organic acids and other injurious products in such oils during service and to substantially reduce piston lacquering, ring-sticking and bearing corrosion in internal combustion engines and the like in which petroleum-base oils are employed as lubricants, by subjecting such oils, after or during service, to the action of at least two alkaline earth metals in elemental or combined inorganic form.

As described and claimed in our co-pending application, Serial No. 219,457, filed July 15, 1938, we have discovered that if petroleum-base oils, either compounded or uncompounded, are heated substantially above normal crank case temperature and passed in contact with a solid selected from the group consisting of the alkaline earth metals and their inorganic compounds, the tendency of the oil to deteriorate during service is reduced and mechanical difficulties, particularly ring-sticking, are inhibited. In another copending application, Serial No. 219,456, filed July 15, 1938, we have described and claimed our discovery that contact masses of alkaline earth metals or inorganic compounds thereof are very effective in preventing deterioration of and corrosion by petroleum base oils containing a soap of an alkaline earth metal even at relatively low temperatures. In a third copending application, Serial No. 219,459, filed July 15, 1938, we have described and claimed our discovery that contact masses of alkaline earth metals or inorganic compounds thereof are likewise effective in preventing deleterious action of petroleum-base oils containing an aluminum soap.

We have discovered also that mixtures containing more than one of the three alkaline earth metals (i. e., calcium, barium and strontium) in elemental or combined inorganic form manifest increased effectiveness in inhibiting deterioration of petroleum-base oils and preventing corrosion thereby, as compared with contact masses containing only one of the alkaline earth metals in combined or elemental form. Thus, we have discovered that a mixture of calcium hydroxide and barium hydroxide is more effective as a corrosion inhibitor and for preventing ring-sticking, piston lacquering and other mechanical difficulties in internal combustion engines than is an equal quantity of either cal-

cium hydroxide or barium hydroxide alone. Similarly, mixtures containing both calcium and strontium in elemental or combined inorganic form or mixtures containing both strontium and barium in elemental or combined inorganic form make a more effective contact mass than do any of the three alkaline earth metals taken alone, whether in elemental form or combined as an inorganic solid.

Our invention, therefore, contemplates the treatment of a petroleum base lubricant by passing it in contact with a mass containing at least two alkaline earth metals in the form of solids selected from the group consisting of the alkaline earth metals and their inorganic compounds. Preferably, the substance is in porous or finely-divided form so that the oil may be passed through it. Thus, the solid or "contact mass" may be in the form of a filter disposed in the lubricating system of a machine, the oil being pumped out of the service zone of the machine, say a crank case of an internal combustion engine, through the filter and back into the service zone. The effectiveness of the contact mass containing at least two alkaline earth metals in combined or elemental inorganic form is increased within limits as the temperature of the oil in contact with the mass is increased.

Our invention will be understood more thoroughly in the light of the following detailed description taken in conjunction with the accompanying single figure which shows in vertical section an appropriate filter containing a contact mass in which at least two alkaline earth metals are present in elemental or combined inorganic form, this filter being connected in the lubricating system of an internal combustion engine, which is shown schematically.

Referring now to the drawing, it will be seen that the filter comprises a cylindrical metal shell 10 having a cover plate 11 bolted to a flange 12 around the top of the shell with a gasket 13 interposed between the flange and the top to insure a tight joint. Disposed concentrically within the shell is a canister 14 made of perforated Monel metal screen or other pervious corrosion-resistant material. The canister is annular in form with an enclosing top portion 15 so that it surrounds a space 16 immediately above an outlet pipe 17. An inlet pipe 18 is provided in the outside of the shell and the space in the shell around the canister is filled with cotton wool 19 or other inert filter medium. The inside of the canister is filled with a pervious mass 20 of an inorganic solid containing in ele-

mental or inorganic combined form at least two of the alkaline earth metals—calcium, strontium and barium. Thus, the canister may be packed with a mixture of twisted calcium and barium foil, or a mixture containing two or more of the alkaline earth metals in combined form, for example, as oxides, carbonates, hydroxides, or carbides. For economic reasons, it is desirable to fill the canister with fine lumps (say 8 to 14 mesh) of calcium hydroxide together with an inorganic compound of strontium or barium or both. Barium and strontium hydroxides should be employed in anhydrous form, because in the crystalline form they lose water at relatively low temperatures.

Oil is withdrawn from the crank case of the engine and by means of a pump forced through the cotton wool and the contact mass 20 to the outlet of the filter, from which point the treated oil is returned to the crank case so that a repeated circulation is set up.

The tendency of the contact mass to escape from the filter is relatively slight. Lumps of the hydroxides of the alkaline earth metals are relatively friable in the air, but when once wetted with oil, there is little tendency for them to break apart. However, the cotton wool or other filter media is provided as a safeguard against the circulation of the hydroxides or other solids through the engine. The cotton also serves to distribute the oil through the contact mass and thus prevent channeling.

As a further precaution against the escape of the contact mass into the engine, it is advisable to soak the mass with oil prior to installing the filter on the engine. This may be done conveniently by pumping oil through the mass, so that fine particles which tend to escape may be removed prior to placing the mass in service in the lubricating system.

As shown, heating means may be provided in the lubricating system preferably ahead of or adjacent to the contact mass so that the oil may be heated to an optimum temperature prior to or during contact with the mass. Within limits established by the thermal stability of the particular oil employed, higher temperatures promote improved action of the contact mass.

Extensive tests indicate that the most desirable contact mass both from the standpoint of econ-

tium or barium. Thus, a contact mass containing two-thirds calcium hydroxide and one-third of either barium hydroxide or strontium hydroxide has given best results in inhibiting ring-sticking and preventing bearing corrosion.

We give below a summary of results obtained with contact masses containing two alkaline earth metals as compared with the results obtained when a mass containing only one of the metals was employed and with results when no contact mass was used. Barium hydroxide alone is slightly inferior to either strontium hydroxide or calcium hydroxide from the standpoint of inhibiting ring-sticking. It is, however, superior to the hydroxides of these other two alkaline metals from the standpoint of preventing bearing corrosion by uncompounded oils. Hence, barium hydroxide alone is superior as a contact mass to either of the other hydroxides taken alone, but as the following results show, is inferior to mixtures containing any two of the alkaline earth metal hydroxides from the standpoint of inhibiting ring-sticking and preventing bearing corrosion, which are the most important factors in the lubrication of modern internal combustion engines.

In all cases, the test procedure was exactly the same except insofar as the contact mass is concerned, and in the temperature of contact. The oil subjected to test was a high-grade uncompounded Pennsylvania lubricating oil adapted for aircraft service. It was circulated through the lubricating system of a gasoline engine, the oil being pumped from the crank case of the engine through a filter and thence returned to the crank case. In Tests 2 to 7, inclusive, the contact mass comprised hydroxide pellets ranging in size from that of a pea down to about 14 mesh. In all cases the total oil in the lubricating system amounted to about 7 liters, and it was circulated through the filter at the rate of about three liters per minute. In each instance the contact mass weighed about 800 to 2000 grams depending on composition. The oil pressure was 15 pounds per square inch in each instance and the pressure drop in the filter ranged from 3 to 8 pounds per square inch. All tests were run for fifty hours, and thereafter the engine was taken down; bearing corrosion was determined; "carbon" deposits were removed, weighed and examined, and the used oil was subjected to analysis.

| Test No.                               | 1        | 2                        | 3                                                               | 4                                                                      | 5                                                                      | 6                                                                           | 7                                                                           |
|----------------------------------------|----------|--------------------------|-----------------------------------------------------------------|------------------------------------------------------------------------|------------------------------------------------------------------------|-----------------------------------------------------------------------------|-----------------------------------------------------------------------------|
| Contact mass used                      | None     | $\text{Ba}(\text{OH})_2$ | $\frac{2}{3}(\text{CaOH})_2, \frac{1}{3}\text{Ba}(\text{OH})_2$ | $\frac{2}{3}\text{Sr}(\text{OH})_2, \frac{1}{3}\text{Ba}(\text{OH})_2$ | $\frac{2}{3}\text{Ca}(\text{OH})_2, \frac{1}{3}\text{Sr}(\text{OH})_2$ | $\frac{2}{3}\text{Ca}(\text{OH})_2, \frac{1}{3}\text{Sr}(\text{OH})_2^{**}$ | $\frac{2}{3}\text{Ca}(\text{OH})_2, \frac{1}{3}\text{Sr}(\text{OH})_2^{**}$ |
| Temp. of contact °F                    | +280-290 | 290                      | 290                                                             | 280-290                                                                | 280-290                                                                | 280-290                                                                     | 240                                                                         |
| Analysis of used oil, percent "Carbon" | 3.310    | 1.69                     | 1.82                                                            | 1.93                                                                   | 2.17                                                                   | 1.88                                                                        |                                                                             |
| Percent tar                            | 0.268    | 0.184                    | 0.204                                                           | 0.236                                                                  | 0.156                                                                  | 0.216                                                                       | 0.160                                                                       |
| Percent asphaltenes                    | 0.148    | 0.048                    | 0.040                                                           | 0.072                                                                  | 0.072                                                                  | 0.144                                                                       | 0.088                                                                       |
| Piston deposits, gms                   | 2.274    | 3.054                    | 3.264                                                           | 1.561                                                                  | 2.8131                                                                 | 1.195                                                                       | 2.902                                                                       |
| Bearing loss, gms:                     |          |                          |                                                                 |                                                                        |                                                                        |                                                                             |                                                                             |
| Cadmium-silver:                        |          |                          |                                                                 |                                                                        |                                                                        |                                                                             |                                                                             |
| A                                      | 2.051    | 0.293                    | 0.023                                                           | 0.094                                                                  | 0.209                                                                  | 0.058                                                                       | 0.437                                                                       |
| B                                      | 2.443    | 0.401                    | 0.068                                                           | 0.119                                                                  | 0.225                                                                  | 0.054                                                                       | 0.499                                                                       |
| Copper lead:                           |          |                          |                                                                 |                                                                        |                                                                        |                                                                             |                                                                             |
| A                                      | 0.405    | 0.358                    | 0.063                                                           | 0.246                                                                  | 0.139                                                                  | 0.105                                                                       | 0.147                                                                       |
| B                                      | 0.404    | 0.322                    | 0.070                                                           | 0.144                                                                  | 0.103                                                                  | 0.084                                                                       | 0.101                                                                       |
| Babbitt:                               |          |                          |                                                                 |                                                                        |                                                                        |                                                                             |                                                                             |
| A                                      | 0.055    | 0.014                    | 0.007                                                           | 0.027                                                                  | 0.012                                                                  | 0.013                                                                       | 0.067                                                                       |
| B                                      | 0.048    | 0.017                    | 0.012                                                           | 0.008                                                                  | 0.010                                                                  | 0.007                                                                       | 0.007                                                                       |
| C                                      | 0.089    | 0.015                    | 0.007                                                           | 0.030                                                                  | 0.066                                                                  | 0.025                                                                       | 0.017                                                                       |
| D                                      | 0.059    | 0.013                    | 0.009                                                           | 0.006                                                                  | 0.011                                                                  | 0.009                                                                       | 0.005                                                                       |
| Ring rating percent free               | 73.3     | 87.0                     | 94.2                                                            | 97.5                                                                   | 75.8                                                                   | 100.0                                                                       | 87.1                                                                        |
| Character of carbon formed             | Hard     |                          |                                                                 |                                                                        | Semi-friable                                                           | Very hard                                                                   | Friable                                                                     |
|                                        |          |                          |                                                                 |                                                                        |                                                                        |                                                                             | Hard                                                                        |

\*Prepared by mixing alkaline earth oxides before hydration.

\*\*Alkaline earth oxides hydrated and dried, then mixed to form mass.

+Temperature of oil as returned to crank case without contact with mass.

omy and of efficiency is one containing about two parts of calcium for each part of either stron-

As the foregoing results show, mixtures containing more than one alkaline earth metal are

to be preferred over contact mass containing only one alkaline earth metal. Bearing corrosion is reduced when using the mixed contact masses with bearings such as cadmium-silver, which are very susceptible to corrosion and also with the relatively corrosion-resistant materials such as babbitt.

The benefits to be obtained by using the mixed contact mass are increased with increased temperature. This is shown by a comparison of the results of Tests 6 and 7. The conditions in these two tests were identical except that the contact temperature in Test 6 was 280-290° F., as contrasted with a contact temperature of 240° F. in Test 7. In consequence of the increased temperature in Test 6, ring-sticking was completely eliminated and corrosion of the three kinds of bearing metals tested was substantially decreased.

A comparison of the results of Tests 5 and 6 shows that it is desirable to mix the alkaline earth hydroxide employed from the mass after hydration of the oxides from which they are formed. In Test 5 the mass was prepared by mixing calcium oxide with strontium oxide and then hydrating and drying the mixture. This procedure is shown to be less satisfactory than the procedure in Test 6 in which the alkaline earth hydroxides are first hydrated and dried and then mixed. Preparation of the contact mass by mixing the alkaline earth oxides prior to hydration is unfavorable in another respect in that a mass thus formed tends to produce hard "carbon" which apparently tends to cause ring-sticking.

The tendency toward forming hard carbon with consequent tendency toward ring-sticking is also increased with a decrease in contact temperature as a comparison of the results of Tests 6 and 7 clearly shows.

We claim:

1. In the operation of a system for lubricating a machine with a petroleum base lubricating oil which involves repeated contacting of said oil from a body thereof with the surfaces to be lubricated and circulation of said oil during service through a treating zone, the improvement which comprises passing the oil in said treating zone through a contact mass containing at least two of the alkaline earth metals in the form of solids selected from the group consisting of the alkaline earth metals and inorganic compounds thereof, at a rate sufficient to bring into contact with said solids an amount of oil equivalent to a substantial part of said body of oil per minute, and controlling the temperature of the oil in said

treating zone to maintain the oil in contact with said contact mass at a temperature approximating 240°-290° F.

2. The process of claim 1 in which the contact mass contains at least two of the alkaline earth metal hydroxides.

3. The process of claim 1 in which the contact mass contains calcium hydroxide and barium hydroxide.

4. The process of claim 1 in which the contact mass contains calcium hydroxide and strontium hydroxide.

5. The process of claim 1 in which the contact mass contains barium hydroxide and strontium hydroxide.

6. The process of claim 1 in which the contact mass contains calcium hydroxide and at least one other alkaline earth hydroxide, the calcium hydroxide being present in an amount exceeding the other alkaline earth metal hydroxide.

7. The process of claim 1 in which the contact mass contains calcium hydroxide and barium hydroxide, the amount of calcium hydroxide present being about twice the amount of barium hydroxide present.

8. The process of claim 1 in which the contact mass contains calcium hydroxide and strontium hydroxide, the amount of calcium hydroxide present being about twice the amount of strontium hydroxide present.

9. The process of claim 1 in which the contact mass contains at least two of the alkaline earth metals hydroxide and in which the oil is brought into contact therewith at a temperature of about 290° F.

10. The process of claim 1 in which the contact mass contains at least two of the alkaline earth metal hydroxides having a particle size ranging from that of a pea to about 14 mesh.

11. In the operation of a system for lubricating a machine with a petroleum base lubricating oil which involves repeated contacting of said oil from a body thereof with the surfaces to be lubricated and circulation of said oil during service through a treating zone, the improvement which comprises heating the oil and passing it in said treating zone through a contact mass containing at least two of the alkaline earth metals in the form of solids selected from the group consisting of the alkaline earth metals and inorganic compounds thereof at a rate sufficient to bring into contact with said solvent an amount of oil equivalent to approximately 40% of said body of oil per minute.

MATTHEW FAIRLIE.  
LEONARD E. BEARE.